

134  
17  
Patented Aug. 4, 19362,049,618  
17  
G

## UNITED STATES PATENT OFFICE

2,049,618

METHOD OF AND COMPOSITION FOR  
TREATING FABRICS TO SEAL THREADS  
THEREOF

Forrest J. Major, Ocean Park, Calif., assignor, by  
mesne assignments, to The Run-Ban Com-  
pany, Steubenville, Ohio, a corporation of  
Ohio

No Drawing. Continuation of application Serial  
No. 724,202, May 5, 1934. This application  
December 22, 1934, Serial No. 758,826

6 Claims. (Cl. 134—17)

This invention relates to a composition particu-  
larly adapted for the washing and cleaning of  
garments, one form of said invention being char-  
acterized by its ability to strengthen delicate  
5 fabrics such as hosiery and other garments,  
whereby so-called "runs" or unraveled areas in  
the fabric are prevented.

Generally stated, the composition of this inven-  
tion has detergent properties which facilitate the  
10 removal of oily and other impurities and also has  
the property of coalescing or sealing individual  
fibres of the fabric, thereby preventing the fibres  
from splitting and eventually breaking.

The so-called runs of silk hose, for example, are  
15 primarily due to a splitting of a thread or fibre  
into a bundle of extremely minute fibre portions  
which then break, causing the cloth to unravel.  
The composition of this invention prevents the  
20 initial splitting of the fibres. Moreover, certain  
forms of the composition impart or retain the  
elasticity of the fibres, thereby preventing the  
fibres from becoming brittle. In addition, when a  
25 thread is composed of a number of undivided  
fibres, the composition causes the individual fibres  
to remain sealed together.

These and other desired properties are im-  
parted to the composition by the conjoint use of  
particular ingredients, as will be described herein-  
after in greater detail.

30 An object of this invention, therefore, is to  
disclose and provide a detergent composition ca-  
pable of strengthening and sealing delicate fibres.

Another object is to disclose and provide an  
aqueous soap composition adapted for use in  
35 washing and cleaning fabrics.

A still further object of the invention is to dis-  
close and provide an aqueous soap composition  
containing sealing and plasticizing agents  
whereby fabrics and/or garments made therefrom  
40 may be cleaned, sealed and strengthened.

The composition of this invention is preferably  
made in concentrated form, which is then used as  
a base in the cleaning and treatment of fabrics,  
garments and the like. The base may contain  
45 water in varying quantities, the quantity of water  
depending upon the concentration desired. In  
use, a small quantity of the base composition is  
added to water or a dilute soap solution in which  
the garments are to be washed. Under certain  
50 conditions it is highly desirable to add a small  
quantity of a dilute or weak acid, such as for  
example, acetic acid, to the washing solution  
before removing the garment from such solution,  
rinsing and drying in the usual manner.

55 The basic ingredients comprise soap and a resin,

oleoresin or wax. In the simplest embodiment of  
the invention, the wax or resin is dissolved in a  
suitable solvent (either aqueous or organic) and  
then incorporated in a strong or concentrated  
5 soap solution, such as a solution containing ap-  
proximately 50% of soap. Whether an organic  
solvent is used or an aqueous solvent depends  
upon the character of the wax or resin. Certain  
resins, such as gum dammar and degummed  
10 resins, can be placed in solution in alkaline aque-  
ous media, such as solutions containing ammonia,  
caustic soda and even relatively weak organic  
bases such as triethanolamine.

When the gums or resins are soluble only in  
organic solvents, such as alcohol, benzol, ben-  
zene, amyl acetate or petroleum hydrocarbon  
solvents, then the resulting product should con-  
tain a sufficient amount of soap so as to form  
an emulsion containing the aqueous soap solu-  
tion in the external phase and the solvent-resin  
15 solution in the internal dispersed phase. Gen-  
erally, the amount of soap should be more than  
twice the amount of resin or wax. When the  
final product is to be in the form of an emulsion,  
the dispersing effect of the aqueous soap solution  
20 may be facilitated by the formation of a tri-  
ethanolamine oleate or other triethanolamine  
soap during compounding.

The following illustrates a composition made  
in accordance with the above disclosure: 1 part 30  
of J & G wax may be melted and dissolved in  
4 parts of water containing 0.25 part of tri-  
ethanolamine; 0.25 part of oleic acid may then be  
added to the hot solution and the resulting mix-  
ture then incorporated in 2 or 3 parts of a soap  
35 solution prepared by dissolving soap in a sub-  
stantially equal weight of water. Any of the so-  
called cold water soaps may be used.

When the above composition is used in wash-  
ing fabrics or garments such as silk hosiery,  
40 a small quantity, say 1 fluid ounce, of the base  
composition is added to 1 quart of water, the  
hose washed therein, and a small quantity, say  
1 or 2 fluid ounces, of a 10% acetic acid solution  
added thereto. The acetic acid appears to exert  
45 a gelatinizing or setting effect upon the wax or  
resin, thereby hardening and strengthening the  
fibres. The hose may then be removed from the  
washing solution and rinsed and dried in the  
usual manner. Instead of acetic acid or vinegar,  
50 other weak acids such as tartaric and citric may  
be used. The acidification is to be carried out  
while the fabrics are in contact with the solu-  
tion, the sealing, coagulation or precipitation of  
55

the resin upon the fibers taking place at that time.

Various waxes and resins may be used in the manner described hereinabove. Particularly good effects have been obtained with some of the synthetic resins, such as the phenol condensation type, the diphenyl chloride type, and colophony. Beeswax, carnauba, copal and so-called Montan wax have also been used.

In order to make certain that the treated fabric or garment retains elastic and pliant properties, it is desirable that the finished composition contain a small proportion of rubber. The following illustrates a composition containing both resin and rubber, together with ranges in which the ingredients may be varied:

| Example              | Range   |          |
|----------------------|---------|----------|
|                      | Percent | Percent  |
| Rubber.....          | 0.5     | 0.1- 2.0 |
| Resin.....           | 4.0     | 1 - 8    |
| Organic solvent..... | 45      | 25 - 60  |
| Oleic acid.....      | 0.25    | 0.1- 5.0 |
| Triethanolamine..... | 4       | 2.5-10   |
| Common soap.....     | 9       | 5 - 20   |
| Water.....           | 37.25   | 25 - 60  |

Differently expressed, the composition may contain about 2 parts of soap and 10 parts of solvent to 1 part of rubber and resin by weight.

In the preferred manner of making up compositions of the hereinabove stated general character, the rubber and resin are preferably dissolved in a suitable organic solvent, such as benzene, benzol, or mixtures containing the hydrocarbon solvents. A portion of the triethanolamine, diluted with water, is then added to the solution of rubber and resin, with agitation. Oleic acid and the remainder of the triethanolamine together with a small proportion of water may then be intermixed to form a triethanolamine soap, which is then diluted with remaining water and intimately mixed with the solution of resin and rubber in the solvent. The desired amount of soap is then dissolved in water, generally by the use of heat, so as to form a concentrated soap solution into which the solvent-triethanolamine soap dispersion is then incorporated. Obviously, the proportion of water appearing in the final composition may vary greatly, depending upon the concentration of the base mixture desired. In addition to the ingredients specified hereinabove, a small quantity of nitrocellulose may be incorporated in the solvents containing the resin and rubber. By the term "rubber" as used herein, reference is made to the unvulcanized coagulated rubber of commerce.

When nitrocellulose is used in the composition, it is used in small quantities comparable to those used for rubber, namely, 0.1% to 2.0% by weight of the composition.

The sealing effect referred to hereinabove which either combines split fibres or individual fibres constituting a thread of material, is particularly pronounced when the composition is used on natural silk and cotton goods. The same sealing effect is not obtained to the same extent on fabrics or threads of cellulose acetate or cellulose substitution derivatives.

When used on silk fibres or fabrics, sealing or cementing action is limited to individual fibres

without detracting from the softness, pliability and strength of the fibres. In the event larger quantities of rubber, resin and/or nitrocellulose than those referred to in the preferred ranges hereinabove, are employed, then the entire fabric may be rendered more moisture or water-resistant. The washing or treating solutions should then contain a much higher proportion of the basic composition than the illustrative proportions referred to hereinabove.

This application is a continuation of Serial No. 724,202.

All changes and modifications coming within the scope of the appended claims are embraced thereby.

I claim:

1. An aqueous soap composition containing a sodium soap and triethanolamine soap, and a solution of resin and coagulated rubber in a solvent, said resin and rubber solution being in stable dispersion in the aqueous soap, said composition containing some free triethanolamine, said solvent being in excess of the soap and said soap being in excess of the rubber and resin by weight.

2. An aqueous soap composition adapted for use in the treatment of fabrics to seal threads thereof, comprising an aqueous soap solution containing from about 0.1% to 2.0% of coagulated rubber, 1% to 8% of resin, 5% to 20% of soap, organic solvents in quantity sufficient to dissolve the rubber and resin and water.

3. An aqueous soap composition adapted for use in the treatment of fabrics to seal threads thereof, comprising an aqueous soap solution containing coagulated rubber, resin, soap, oleic acid, triethanolamine in excess of that capable of combining with oleic acid, organic solvents in quantity sufficient to dissolve the rubber and resin and water, said solvent being in excess of the soap and said soap being in excess of the rubber and resin by weight.

4. An aqueous soap emulsion having an organic solvent dispersed therein, said solvent containing resin and coagulated unvulcanized rubber in solution therein, said solvent being in excess of the soap and said soap being in excess of the rubber and resin by weight, said soap emulsion being adapted to seal and strengthen threads of silken fabrics immersed therein in the presence of added acid.

5. A method of strengthening and sealing threads of silken fabrics, which comprises contacting fabrics with a dispersion of a soap emulsion containing an organic solvent dispersed therein, said solvent having resin and coagulated rubber in solution, said dispersion containing not more than about 2% of rubber and 8% of resin, and then acidifying said soap dispersion while in contact with said fabric.

6. An aqueous emulsion containing an organic solvent dispersed in a soap solution, said organic solvent containing coagulated rubber and resin dissolved therein, said emulsion containing the ingredients in the ratio of about 2 parts of soap and 10 parts of solvent to 1 part of rubber and resin by weight, said emulsion being adapted to seal and strengthen threads of silken fabrics immersed therein in the presence of added weak acids.

FORREST J. MAJOR.